

## UNITED STATES PATENT OFFICE

2,347,814

## LUBRICANT

Truman E. De Villiers, Okmulgee, Okla., assignor  
to Cities Service Oil Company, Bartlesville,  
Okla., a corporation of Delaware

No Drawing. Application November 7, 1942,  
Serial No. 464,897

## 14 Claims. (Cl. 252—34)

This invention relates to lubrication and to lubricants therefor. More particularly the invention relates to the stabilization of crank case lubricants with addition agents adapted to inhibit oxidation of the lubricating oil, prevent corrosion of crank case bearing surfaces, and increase the load-carrying capacity of the lubricating oil.

Various compounds and compositions have been proposed for the stabilization of lubricating oils, and it is well-known that unprotected mineral lubricating oils, especially in contact with air and at elevated temperatures become dark and produce sludge. Many bearing metals and bearing compositions catalyze the deterioration of unprotected crank case lubricants under the conditions involved in their use. Solvent refined petroleum lubricating oils seem to be somewhat more susceptible to deterioration in crank cases than petroleum lubricants produced by other refining methods. In many cases it is the practice to use separate agents to inhibit oxidation and provide extreme pressure characteristics. However, according to the present invention an addition agent has been discovered which inhibits oxidation, prevents corrosion of bearing surfaces, and also increases the load-carrying capacity of the lubricating oil.

The primary object therefore of the present invention is to provide an effective method of lubrication and to provide a stabilized lubricant of relatively high load-carrying capacity therefor.

Another object of the invention is to provide an effectively stabilized lubricating oil for the crank cases of automobiles and Diesel engines.

These and other objects are accomplished in accordance with the present invention by mixing and dissolving a relatively small proportion of an organic tertiary amine phosphite in a mineral lubricating oil normally subjected to deterioration in the presence of oxygen, and normally corrosive to crank case bearings.

It has been previously proposed that certain amine derivatives containing phosphorus be used as addition agents for lubricating oils as shown by Patent No. 2,146,543 and Patent No. 2,146,584, both granted on February 7, 1939, but it appears that all of the compounds disclosed in these patents involve a P—N linkage. The organic tertiary amine phosphites of the present invention on the contrary all contain the linkage P—OR—N, (R being an alkyl, aryl or alkaryl group or radical). Compounds of this type have been found to be unusually effective in stabiliz-

ing crank case lubricating oils, preventing bearing corrosion, and in increasing the load-carrying capacity of the lubricating oil.

The features of the invention will be illustrated more in detail by reference to certain specific examples and data. The method of manufacturing certain representative compounds are illustrated in the following examples:

## Example No. 1

10 Tri-triethanolamine phosphite, in which each triethanolamine group is attached to phosphorus with an O—P linkage, was made from triethanolamine and phosphorus trichloride. 100 cc. of anhydrous ether, 400 cc. of anhydrous benzene, and 45 grams of triethanolamine were placed in a 1000 cc. three-necked flask equipped with a reflux condenser including a HCl trap, a mercury sealed stirrer, and a separatory funnel. A mixture of 13.7 grams of phosphorus trichloride in 100 cc. of anhydrous ether was slowly introduced into the flask through the separatory funnel. Agitation of the materials in the flask was continued throughout the addition of the phosphorus trichloride and for one hour afterward.

15 During this time, a white precipitate was formed and was separated out from the solvents. The precipitate was dissolved in about 500 cc. of alcohol containing sufficient alcoholic KOH to neutralize the HCl formed. Most of the alcohol was then removed from the mixture by distillation, and the resulting KCl filtered off. The product was finally freed of alcohol and water in a desiccator under high vacuum at a temperature of about 160° F. The product was found to contain approximately the calculated proportions of phosphorus and nitrogen and to be free of chlorine. Analysis showed a phosphorus content of 5.76%, whereas the calculated value is 40 6.53%. The nitrogen found in the compound was 8.70% while the calculated value is 8.84%.

## Example No. 2

45 Tri-ethanodiethylamine phosphite, in which each amino group is attached to phosphorus by an O—P linkage, was made from phosphorus trichloride and ethanoldiethylamine. The apparatus used was the same as that employed in Example No. 1, 300 cc. of anhydrous benzene being introduced into the flask, after which agitation was started and 80 grams of ethanoldiethylamine added. Thereafter while the agitation was continued, a mixture of 50 cc. of anhydrous benzene and 10 grams of phosphorus trichloride was slowly added to the mixture in

the flask. The refluxing and stirring was continued for two hours, after which about half the benzene was distilled off. The remainder of the reaction mixture in the flask was then dissolved in alcoholic KOH containing sufficient KOH to neutralize the HCl formed. The resulting KCl precipitate was filtered off and the filtrate transferred to a distillation flask where most of the solvent was stripped off. More benzene was added to the mixture in the distilling flask, about a liter in all, to completely remove the water. This point was indicated when the distillate came over clear. During the distilling operation care was exercised to avoid complete removal of benzene and overheating of the material in the flask, the last traces of benzene being removed, however, along with unreacted amine in a vacuum desiccator at about 160° F. The product was found to contain 7.89% of phosphorus where the calculated value is 8.18%, and to contain 11.53% of nitrogen where the calculated value is 11.08%.

*Example No. 3*

Dicresyl mono-triethanolamine phosphite was prepared from phosphorus trichloride, o-cresol and triethanolamine. The apparatus used was the same as that described in Example No. 1, 400 cc. of anhydrous benzene and 54.8 grams of phosphorus trichloride being first introduced into the flask, after which 86.4 grams of o-cresol were added at a fairly rapid rate. Heating was begun and the mixture was refluxed until evolution of HCl stopped, which took about one hour. The reflux condenser was removed from the flask and rearranged for the removal of the solvent by distillation. The distillation of the benzene carried off the remaining HCl gas which was separated from the condensed benzene, the latter being returned to the flask to effect the stripping out of the HCl from the reaction mixture comprising dicresyl phosphorus chloride and benzene.

The reaction mixture in the flask was reduced so that it contained only about 200 cc. of benzene and was then added to another flask containing 200 cc. of benzene and 55 grams of triethanolamine. This mixture was refluxed with agitation for one hour. An oily layer separated at the bottom of the mixture, and was removed. The water and benzene content of the product was removed in a vacuum desiccator at about 160° F. The product was found to contain no halogen, 8.88% phosphorus, and 1.39% nitrogen. The calculated values for phosphorus and nitrogen are 7.89% and 3.56% respectively. The high value for phosphorus and the low value for nitrogen indicates that the product is a mixture and probably contains compounds in which two, or possibly three dicresyl phosphite groups,  $-\text{P}(\text{OR})_2$ , are attached to a single triethanolamine group by  $\text{O}-\text{P}$  linkages. Such compounds may be illustrated by the general formula:



and



The effectiveness of the addition agents of the present invention is illustrated by the data produced below in tests carried out on the compounds of the foregoing examples. These compounds were blended with a Mid-Conti-

10 nent solvent extracted 30 S. A. E. lubricating oil, having a Saybolt Universal viscosity at 210° F. of 62.7 seconds. The following table shows the results obtained on the Underwood testing apparatus, the oil along being run only 20 hours as against 50 hours for the blends. In the table the addition agent in each blend is referred to by the number of the example above, by which it was produced.

|    |                                                 | Oil alone | Oil with 0.2% of No. 1 | Oil with 0.5% of No. 2 | Oil with 0.5% of No. 3 |
|----|-------------------------------------------------|-----------|------------------------|------------------------|------------------------|
| 15 | Duration of test                                | 20 hrs.   | 50 hrs.                | 50 hrs.                | 50 hrs.                |
|    | Copper baffle:                                  |           |                        |                        |                        |
|    | Corrosion                                       | Medium    | Very light             | Medium                 | Very light.            |
|    | Lacquer deposit                                 | do        | do                     | do                     | None.                  |
| 20 | Heater rods: Corrosion.                         | do        | None                   | Light                  | Do.                    |
|    | Bearings (cadmium-silver): loss in weight, gms. | 1.658     | 0.000                  | 0.067                  | 0.000                  |
|    | Condition of oil sludge, mg./10 g.:             |           |                        |                        |                        |
|    | 10 hrs.                                         | 11        | 13                     | 14                     | 11.                    |
|    | 20 hrs.                                         | 1,099     | 17                     | 15                     | 10.                    |
|    | 30 hrs.                                         |           | 16                     | 18                     | 11.                    |
|    | 40 hrs.                                         |           | 16                     | 14                     | 9.                     |
|    | 50 hrs.                                         |           | 14                     | 16                     | 10.                    |
| 25 | Neutralization No. (electrometric at pH 11.0):  |           |                        |                        |                        |
|    | 10 hrs.                                         | 13.2      | 4.0                    | 4.0                    | 0.2.                   |
|    | 20 hrs.                                         | 31.2      | 5.9                    | 9.0                    | 0.3.                   |
|    | 30 hrs.                                         |           | 7.8                    | 16.2                   | 0.3.                   |
|    | 40 hrs.                                         |           | 15.6                   | 16.4                   | 0.4.                   |
|    | 50 hrs.                                         |           | 19.4                   | 19.9                   | 0.4.                   |
| 30 | Viscosity-S. U. @ 210° F.:                      |           |                        |                        |                        |
|    | 10 hrs.                                         | 92.5      | 64.1                   | 68.3                   | 63.3.                  |
|    | 20 hrs.                                         | 365.0     | 65.9                   | 72.1                   | 63.8.                  |
|    | 30 hrs.                                         |           | 70.0                   | 75.4                   | 64.2.                  |
|    | 40 hrs.                                         |           | 78.4                   | 80.3                   | 64.6.                  |
|    | 50 hrs.                                         |           | 85.7                   | 85.8                   | 65.4.                  |

Other portions of the same oil and of the compositions tested in the Underwood oxidation apparatus were also tested in the Cornell (Falex) testing machine with the results shown in the following table:

|    |                          | Oil alone | Oil with 0.2% of No. 1 | Oil with 0.5% of No. 2 | Oil with 0.5% of No. 3 |
|----|--------------------------|-----------|------------------------|------------------------|------------------------|
| 45 | Temperature:             |           |                        |                        |                        |
|    | Start, °F.               | 98        | 90                     | 95                     | 95                     |
|    | Finish, °F.              | 178       | 240                    | 250                    | 272                    |
| 50 | Jaw load-torque @—       |           |                        |                        |                        |
|    | 250 lbs.                 | 3         | 3                      | 3                      | 2                      |
|    | 500 lbs.                 | 7         | 8                      | 5                      | 9                      |
|    | 750 lbs.                 | 12        | 12                     | 13                     | 10                     |
|    | 1,000 lbs.               | 18        | 16                     | 21-70                  | 16                     |
|    | 1,250 lbs.               | Seized    | 22                     | 26                     | 21                     |
|    | 1,500 lbs.               |           | 25                     | 33                     | 26                     |
|    | 2,000 lbs.               |           | 30                     | 42                     | 31                     |
|    | 2,500 lbs.               |           | 31                     | 50                     | 41                     |
|    | 3,000 lbs.               |           | 37                     | 63                     | 51                     |
|    | 3,500 lbs.               |           | 42                     | 67                     | 63                     |
|    | 4,000 lbs.               |           | 54                     | 73                     | 74                     |
|    | 4,500 lbs.               |           | 80                     | 90                     | 78                     |
| 55 | Failure at . . . pounds. | 1,250     | No                     | 11,000                 | No                     |
|    | Wear:                    |           |                        |                        |                        |
|    | Pin                      | Med.      | Med.                   | Scar                   | Slight                 |
|    | Bushings . . . inches.   | 1/16      | 1/16                   | 1/16                   | 1/16                   |

<sup>1</sup> Slight seizure producing scar followed by carrying full load.

In the Underwood tests on the solvent extracted oil without the addition agent, the bearing corrosion started before ten hours had elapsed, and had progressed considerably at the ten-hour period. The ability of the compounds of the present invention to protect the bearings against corrosion is strikingly illustrated by the complete protection obtained in spite of the fact that the neutralization numbers went up considerably in the cases of agents numbers 1 and 2, as the tests proceeded.

The addition agents of the present invention are especially effective with, and are preferably

used with petroleum lubricating oils refined by solvent extraction methods. They are also useful and beneficial in any crankcase lubricant regardless of its origin or of the method by which it is refined. The proportion of the addition agent may vary from 0.05% to 5% of the lubricating oil stock and may be admixed therewith in the form of a concentrate in a mutual solvent. In certain cases the use of a concentrate in a solvent is preferred because certain of the compounds such as those containing a number of OH radicals are not very soluble in the lubricating oil stock. So far, however, no difficulty has been encountered in dissolving the relatively small proportions as for example 0.5% of the agent in the lubricating oil.

From the foregoing description of the invention taken in connection with the examples and data presented, it will be apparent that since all compounds coming within the scope of the invention are tri-valent phosphites and include the group P-ORN, the number of possible compounds is rather limited. However, certain variations are possible as illustrated by the compounds of the examples. The compound may include the group —ORNR'<sub>2</sub>, either one, two or three times, and that where only one or two such groups are included in the compound, it may also include respectively two or one —OR group attached to phosphorus. The R' radicals in this compound may be alkyl, aryl, alkaryl, hydroxy alkyl, hydroxy aryl, or hydroxy alkaryl. In certain special instances, the compound may be a polymer-type derivative containing two or more of the groups P-ORNR'<sub>2</sub> linked together in the manner indicated above in Example No. 3.

The examples and data given above are for purposes of illustration, and it is not intended that the invention shall be limited thereby, the invention being defined by the claims and limited only by the scope of the invention and the prior art.

Having thus described the invention in its preferred form, and illustrated the same in connection with certain specific examples, what is claimed as new is:

1. A crank case lubricating oil composition comprising a relatively large proportion of a solvent refined mineral lubricating oil normally tending to deteriorate and corrode the bearings of the crank case under conditions of normal use and a relatively small proportion of an oil-soluble stabilizing agent admixed therewith sufficient to inhibit such deterioration and prevent such corrosion, said agent comprising a tri-trialkanolamine phosphite, said composition being further characterized by a relatively high stability toward deterioration by oxidation under the conditions of normal use in the presence of the metals of the crank case.

2. A crank case lubricating oil composition as defined by claim 1 in which said phosphite is tri-triethanolamine phosphite.

3. A lubricating oil composition comprising a relatively large proportion of a refined mineral lubricating oil having dissolved therein a relatively small but sufficient proportion of an oxida-

tion and corrosion inhibiting agent, comprising an organic phosphite containing the group P-ORNR'<sub>2</sub> in which R is an organic radical selected from the group consisting of alkyl, aryl, and alkaryl radicals, and R' is an organic radical selected from the group consisting of alkyl, aryl, alkaryl, hydroxy alkyl, hydroxy aryl and hydroxy alkaryl radicals.

4. A lubricating oil composition as defined by claim 3 in which said phosphite has the general formula P(ORNR'<sub>2</sub>)<sub>3</sub>.

5. A lubricating oil composition as defined by claim 3 in which said phosphite has the general formula ROP(ORNR'<sub>2</sub>)<sub>2</sub>.

6. A lubricating oil composition as defined by claim 3 in which said phosphite has a general formula (RO)<sub>2</sub>P-ORNR'<sub>2</sub>.

7. A lubricant comprising a relatively large proportion of a mineral lubricating oil and a relatively small but effective proportion of a product of the reaction between phosphorus trichloride and a tertiary organic amine as an oxidation inhibitor.

8. A lubricant comprising a relatively large proportion of a mineral lubricating oil refined by solvent extraction and a relatively small but effective proportion of an oxidation inhibitor comprising the reaction product produced by reacting phosphorous trichloride with a tertiary organic amine containing an OH group included in at least one of its organic groups.

9. A lubricant comprising a relatively large proportion of a mineral lubricating oil and a relatively small but effective proportion of an oxidation inhibitor comprising an organic phosphite containing the group P-ORNR'<sub>2</sub>, in which R is an organic radical selected from the group consisting of alkyl, aryl, and alkaryl radicals, and R' is an organic radical selected from the group consisting of alkyl, aryl, alkaryl, hydroxy alkyl, hydroxy aryl and hydroxy alkaryl radicals.

10. A crank case lubricant consisting almost entirely of a refined mineral lubricating oil and a relatively small but effective proportion of an oxidation and corrosion inhibitor comprising triethanolamine phosphite.

11. A stabilized crank case lubricant consisting essentially of a refined mineral lubricating oil having dissolved therein from 0.02% to 5% of an organic tri-ester of tri-valent phosphorus, in which at least one ester group is an organic tertiary amine.

12. A lubricant as defined by claim 11 in which at least one ester group is o-cresol.

13. A lubricant comprising a relatively large proportion of a mineral lubricating oil and a relatively small but sufficient proportion of an oxidation and corrosion inhibitor comprising a tri-ester of phosphorous acid in which each of the ester groups is an organic tertiary amine.

14. A lubricant comprising a relatively large proportion of a mineral lubricating oil and a relatively small but sufficient proportion of an oxidation and corrosion inhibitor comprising a tri-triethanolamine phosphite.

TRUMAN E. DE VILLIERS.